

## UNITED STATES PATENT OFFICE.

JOHN WESLEY MARDEN, OF EAST ORANGE, NEW JERSEY, ASSIGNOR TO WESTINGHOUSE LAMP COMPANY, A CORPORATION OF PENNSYLVANIA.

## ACTIVATION OF REFRACTORY METAL FILAMENTS.

No Drawing.

Application filed March 31, 1923. Serial No. 629,190.

This invention relates to the activation of material for electron-emission purposes and more particularly to the use of a halide of thorium or the like and aluminum for such purposes.

An object of my invention is the preparation of filamentary material coated with metallic thorium, whereby good electron emissivity is imparted thereto.

Another object of my invention is the application of a mixture of halide of thorium and finely powdered aluminum, whereby when the same is heated, metallic thorium is developed thereon to give good activation.

A further object of my invention is the use of thorium fluoride or an anhydrous double fluoride of thorium and an alkali metal, mixed with powdered aluminum, for activation purposes, either by applying the mixture directly to a filament or cathode for electron-emission or by application to a component part of an electron device, for example, the plate or anode of a radio tube and transfer of thorium developed thereon by heat, to an adjacent filament.

A still further object of my invention is the utilization of a halide of a refractory metal, such as thorium, uranium, zirconium or the like, preferably the fluoride or double fluoride with an alkali metal, mixed with powdered aluminum for the preparation of the respective refractory metal for activation or other purposes.

Other objects and advantages of the invention will be made apparent upon reading the following description.

Various methods have been employed for developing thorium on filamentary material in evacuated vessels, for electron-emission purposes.

In the copending application of C. T. Ulrey, Serial No. 577,021, filed July 24, 1922, manufacture of electron-emitting devices and the like and assigned to the Westinghouse Lamp Company, is disclosed a method of applying thorium to the electron-emitting filament in a radio tube or the like by applying a piece of metallic thorium to the plate thereof, applying finely divided thorium

thereon in the form of paint or by making said plate of thorium, in whole or in part. A portion of said thorium on the plate is then transferred to the electron-emitting filament in the tube by highly heating the plate in any desired manner, for example, by electron bombardment or high-frequency induction, to cause a transfer of thorium from the plate to the filament.

In my copending application Serial No. 629,189, filed March 31, 1923, electron devices and their manufacture, and assigned to the Westinghouse Lamp Company, is disclosed a method of activation, similar to that of the Ulrey application above referred to, except that, instead of using free thorium on the plate, a mixture of thoria, or other thorium compound, and carbon may be applied thereon, with or without a clean-up agent, such as aluminum or magnesium. Such a mixture on the plate is subsequently heated to cause a liberation of thorium and transfer thereof, at least in part, to the electron-emitting filament.

Both of the aforementioned methods are desirable but the former entails the use of metallic thorium which is expensive and difficult to keep in an unoxidized or uncontaminated condition. The latter obviates the use of expensive metallic thorium but entails the use of such material as carbon which results in the liberation of gaseous carbon compounds which are undesirable as part of the residual atmosphere in the bulb and necessitate an extra quantity of clean-up material for their elimination.

According to my present invention, I avoid the use of expensive metallic thorium and the generation of undesirable gaseous carbon compounds by using a salt of thorium which is reducible by aluminum or other desirable metal. The aluminum may serve the double purpose of reducing the thorium compound used and cleaning up residual gases in the bulb.

It has been found that the class of salts of thorium most suitable for the purpose are the halides, of which the fluoride is preferred. Although thorium tetra-fluoride ( $\text{ThF}_4$ ) may be employed, for certain reasons a double

fluoride of thorium and an alkali metal, for example, potassium-thorium fluoride, having the formula  $KThF_5$  or  $K_2ThF_6$  is preferred. Such material, preferably mixed with an excess of finely divided aluminum, may be applied or gettered on a tungsten wire, for example, in any desired manner, using cryolite mixed therewith as a binder, if desired, or painted on or attached to the plate for a radio tube and sealed into a bulb. After exhausting the bulb, the wire or filamentary cathode therein may be activated by heating the same, if the mixture was applied directly thereto, or if the mixture was merely applied to the plate adjacent thereto, by heating said plate until thorium is liberated therefrom and transferred to the filament.

In the following description, my invention will be explained more in detail.

It is known in metallurgy that thorium chloride, for example, may be reduced by sodium but neither thorium chloride nor sodium can be exposed to the air without contamination, nor can they be gettered or applied to a wire or filament in any known manner without complete oxidation of both the sodium and the thorium chloride.

In my copending application Serial No. 498,397, filed September 3, 1921, the preparation of metals and their halides and assigned to the Westinghouse Lamp Company, is disclosed a method for the production of the anhydrous halides of refractory metals, including thorium, by the treatment of a hydrous salt of such a metal with an agent, for example, ammonium chloride, which will displace the water from such salt. Such method is particularly adapted for producing thorium chloride, which may then be used for the production of other halides of thorium, more particularly adaptable for practicing the present invention. For example, thorium chloride, produced in any desired manner or according to the method disclosed in my referred-to application, may be fused with a small excess of potassium fluoride to produce potassium-thorium fluoride ( $KThF_5$  or  $K_2ThF_6$ ) according to one of the following equations:—



The exact proportions in which these salts are fused, is not essential, as a small excess of potassium fluoride makes no difference. After complete fusion, the mass is cooled, powdered and the soluble constituents thereof dissolved out by water. The excess of potassium fluoride dissolves away, leaving the double thorium salt desired, which is insoluble in water and dilute acids. This should then be ground, as fine as possible, and mixed with aluminum, which is preferably in a finely divided condition and in excess of that needed to completely reduce the thorium con-

tained in the compound according to the following equation:—



Although double salts of thorium and potassium have been mentioned, it is obvious that other double salts may be employed instead, for example, double salts of thorium and sodium. On the other hand, it is not necessary to use a double halide of thorium, as thorium tetra-fluoride may be used directly. This salt may be prepared by precipitation from a water solution of the chloride, but is not always free from oxide when made in this way. It is, however, suitable for activation purposes.

The double halide of thorium and an alkali metal or the halide of thorium which, as heretofore mentioned, it is desired to use, may then be mixed in the form of a dry powder with finely divided aluminum and applied either to a filament or wire to be activated or to a plate intended to be used in cooperation therewith. The proportion of aluminum and the halide salt used, does not have to be exact, but it is preferable that there shall be an excess of aluminum over that needed to reduce the thorium in said salt to the metal, for the purpose of cleaning up residual gases in the bulb, although, of course, if such excess is not employed, some other clean-up agent, for example, magnesium, may be used instead.

The mixture of potassium-thorium fluoride and aluminum, for example, may then be applied to a filament or wire of tungsten or the like, which it is desired to use for electron-emitting purposes, either as an aqueous suspension or paste or in the form of a paint with some suitable vehicle or binder, such as an amyl acetate solution of nitrocellulose or with cryolite, in a manner similar to that for holding thoria and the like on a filament, and described and claimed in the copending application of MacRae and Richardson, Serial No. 566,847, filed June 8, 1922, getters and the application thereof and assigned to the Westinghouse Lamp Co. The filament may then be sealed into a bulb and heated to incandescence until the thorium is reduced, as may be determined by noting the increase in the thermionic current therefrom, in any desired manner, or in the manner disclosed in the application of C. T. Ulrey, before referred to.

Instead of applying the mixture directly to the filament, the same may be applied instead, to a plate or anode intended to be used in the bulb in cooperation with, and adjacent to said filament. After sealing both the filament and the coated plate into a bulb and evacuating said bulb, the filament may be activated by heating the plate in any desired manner, for example, by electron bombardment or high-frequency induction, until the

filament becomes activated to a suitable degree by a transfer of liberated thorium thereto from the plate in a manner similar to that disclosed in the aforementioned Ulrey application.

The excess of aluminum serves to clean up residual gases in the bulb, making it possible to use a cold exhaust as disclosed in the co-pending application of H. C. Rentschler, Serial No. 582,261, filed August 16, 1922, vacuum devices and method of exhausting the same and assigned to the Westinghouse Lamp Company.

It is obvious that the foregoing is a disclosure of means for introducing a metal into a vacuum device, or even an evacuated device containing an inert gas at reduced pressure, for activation or for any other desired purpose. For example, if it is desired to introduce thorium, uranium, zirconium, calcium or any element, for that matter, a mixture of a compound or salt thereof with a reducing agent, such as aluminum, may be applied to the plate of a radio tube, for example, or even upon an auxiliary plate in a lamp. The mixture is subsequently heated, as aforescribed, the compound is reduced and the desired metal, for example, is liberated for accomplishing the purpose, whether that be the activation of an electron-emitting filament, the cleaning-up of residual gases for combination with which it is particularly adapted, or the purification of an inert gas filling.

Although thorium has been mentioned as the preferred activating material, electron-emitting filaments may be activated by other metals, having good electron-emission properties, for example, uranium, zirconium and the like, in the manner disclosed for activating by means of thorium and I do not wish to be restricted entirely to thorium, but desire that it be understood that such modifications as fall within the scope of the appended claims pertain to my invention.

What is claimed is:

1. The method of activating, in a vacuum, a refractory filament for electron-emission purposes comprising placing adjacent thereto, a mixture of a halide of thorium and powdered aluminum and heating said mixture to cause metallic thorium to be liberated and form on the filament.

2. The method of increasing the emissivity of a filamentary metal cathode comprising placing adjacent thereto, a mixture of a double halide of thorium and an alkali metal with finely divided aluminum and heating said mixture to cause a reduction of said thorium compound and a formation of thorium on the cathode.

3. The method of activating a refractory filament for electron-emission purposes comprising applying thereto, a mixture of a halide of a metal of good electron-emission

properties and powdered aluminum, enclosing the same in an evacuated vessel and heating the filament to cause a reaction in the applied mixture with a liberation of the free metal on the filament.

70

4. The method of activating a refractory metal filament for electron-emission purposes, comprising applying thereto, a mixture of a fluoride of thorium and aluminum with a suitable binding material, enclosing the same in an evacuated envelope and heating the filament to cause a reduction and liberation of free metallic thorium thereon.

75

5. The method of activating a refractory metal filament for electron-emission purposes comprising applying thereto, a mixture of potassium thorium fluoride and powdered aluminum held thereon by means of a suitable binding material, enclosing the same in an evacuated envelope and heating the filament to cause an interaction between the thorium compound and the aluminum with the liberation of free metallic thorium on the filament.

80

6. An electron device comprising an evacuated vessel having sealed therein a cathode, an anode and a mixture of a halide of thorium and aluminum applied to at least one of said elements.

85

7. An electron device comprising an evacuated envelope into which is sealed a filament and a plate, to one of which has been applied a mixture of a halide of a metal suitable for electron-emission purposes, and a metallic reducing agent.

90

8. An electron device comprising an evacuated envelope enclosing a filament and a plate cooperating therewith and adjacent thereto and a mixture of a fluoride of thorium and aluminum applied to one of said elements.

95

9. An electron device comprising an evacuated vessel enclosing an electron-emitting cathode and a cooperating anode, one of said elements having applied thereto, a mixture of potassium-thorium fluoride and an excess of aluminum, whereby said aluminum serves the double function of reducing the thorium salt to liberate thorium and to clean up residual gases in the vessel.

100

10. An electron device comprising an evacuated envelope into which is sealed a cathode and an anode, and a mixture of a fluoride of thorium and powdered aluminum applied to said cathode.

105

11. An electron device comprising an evacuated envelope enclosing a filamentary cathode coated with a mixture of potassium-thorium fluoride and an excess of aluminum, and an anode cooperating therewith.

110

12. An electron device comprising an evacuated vessel enclosing a filament and a cooperating electrode coated with a mixture of thorium fluoride and aluminum and held thereon by means of a suitable binding material.

115

13. The method of introducing thorium

120

into an evacuated device comprising mixing potassium thorium fluoride with powdered aluminum, applying said mixture to an element in the device and heating to cause a reaction with the liberation of free thorium therein.

14. An evacuated device comprising a vessel enclosing a mixture of potassium thorium

fluoride and aluminum, said mixture being applied on a conductive element in the device 10 whereby the same may be heated to effect a reaction in the mixture.

In testimony whereof, I have hereunto subscribed my name this 30th day of March, 1923.

JOHN WESLEY MARDEN.